# EUROPEAN PATENT SPECIFICATION

(11) **EP 1 378 582 B1**
(45) Date of publication and mention of the grant of the patent: **20.10.2004**
(21) Application number: 03253539.5
(22) Date of filing: 04.06.2003
(51) Int. Cl.: C22F 1/18

(54) **A method of heat treating titanium aluminide**
Verfahren zur Wärmebehandlung von TiAl-Legierungen
Procédé pour le traitement thermique des alliages de TiAl

(30) Priority: 05.07.2002 GB 0215563
(43) Date of publication of application: 07.01.2004
(73) Proprietor: ROLLS-ROYCE plc, London, SW1E 6AT (GB)
(72) Inventor: Hu, Dawei, Birmingham B31 2DA (GB)
(74) Representative: Gunn, Michael Alan

(56) References cited:
- US-A- 5 417 781
- US-A- 5 653 828
- US-A- 5 746 846
- SEMIATIN S L ET AL: "HOMOGENIZATION OF NEAR-GAMMA TITANIUM ALUMINIDES: ANALYSIS OF KINETICS AND PROCESS SCALEUP FEASIBILITY" METALLURGICAL TRANSACTIONS A. PHYSICAL METALLURGY AND MATERIALS SCIENCE, METALLURGICAL SOCIETY OF AIME. NEW YORK, US, vol. 24A, no. 6, 1 June 1993 (1993-06-01), pages 1295-1306, XP000369947

## Description

The present invention relates to a method of heat-treating titanium aluminide and in particular to a method of heat-treating.

There is a requirement to refine the microstructure of a titanium aluminide alloy, in particular cast titanium aluminide alloy, which does not involve hot working of the titanium aluminide alloy.

It is known to use six to eight rapid heating and rapid cooling cycles of a titanium aluminide alloy to obtain satisfactory fineness of the microstructure, as disclosed by Wang JN, Xia K in Intermetallics 2000, 8, 545. But this is only practical on a laboratory scale. The rapid heating and rapid cooling is beyond the ability of conventional heat treatment facilities. In order to achieve rapid heating and rapid cooling of a titanium aluminide component, the size of the titanium aluminide component is limited and cracks may be produced in an irregular shaped titanium aluminide component.

It is also known to use a first long term soak at a sub alpha transus temperature and a second short term soak at a temperature just above the alpha transus temperature followed by furnace or air cooling of a titanium aluminide alloy, as disclosed by Yang J, Wang JN, Wang Y, Xia QF and Zhang B in Intermetallics 2001, 9, 369. However, the first long term soaking temperature has to be as close to the alpha transus temperature as possible in order to minimise the soaking time. During the first long term soaking the original lamellar microstructure transforms into granular gamma and alpha with a high volume fraction of the alpha phase. The remaining gamma grains act as pinning points to prevent the rapid growth of alpha phase. The second short term soaking temperature has to be above the alpha transus temperature and as close as possible to the alpha transus temperature and the second short term soaking should be as short as possible. This heat treatment requires precision control and rapid heating to the second short term soaking temperature. The aim is to leave the titanium aluminide alloy in the alpha phase field for the shortest possible time to prevent excessive alpha grain growth but this is difficult to realise in a production environment.

Furthermore it is known to provide rapid heating at a rate of about 1500°Cs⁻¹ to a temperature above the alpha transus temperature, a short holding of about 5 minutes at this temperature and normal cooling to produce a fully lamellar refined microstructure in a titanium aluminide alloy, as disclosed by Salishnov GA, Imayev RM, Kuznetsov AV, Shagiev MR, Imayev VM, Shenkov ON, Froes FH, In Kim Y-W, Dumiduk DM, Loretto MH, editors of Gamma Titanium Aluminides 1999, Warendale, PA:TMS, 1999, p291. However, the rapid heating rate required is difficult to achieve using a conventional furnace and the very short holding time is difficult to control. Additionally prolonged holding at a temperature above the alpha transus temperature results in rapid growth of alpha grains, which limits the use of this technique in industrial applications. US-A-5 746 846 discloses a method to produced a fine grained gamma phase, nearly lamellar, microstructure by hot working the alloy in the range of 700°C to Tₐₗₚₕₐ +20°C followed by annealing at Tₐₗₚₕₐ -20°C to Tₐₗₚₕₐ -1°C.

Accordingly the present invention seeks to provide a novel method of heat-treating titanium aluminide alloy which reduces, preferably overcomes, the above-mentioned problems.

Accordingly the present invention provides a method of heat-treating titanium aluminide alloy, the titanium aluminide alloy having a single alpha phase field and being capable of producing a massively transformed gamma microstructure, the method comprising the steps of
(a) heating a titanium aluminide alloy to a temperature above the alpha transus temperature,
(b) maintaining the titanium aluminide alloy at a temperature above the alpha transus temperature in the sinqle alpha phase field for a predetermined time period,
(c) cooling the titanium aluminide alloy from the single alpha phase field to produce a massively transformed gamma microstructure,
(d) heating the titanium aluminide alloy to a temperature below the alpha transus temperature in the alpha and gamma phase field,
(e) maintaining the titanium aluminide alloy at the temperature below the alpha transus temperature for a predetermined time period to precipitate alpha plates in the massively transformed gamma microstructure such that a refined microstructure is produced in the titanium aluminide alloy,
(f) cooling the titanium aluminide alloy to ambient temperature.

Preferably in step (b) the predetermined time period is up to 2 hours.

Preferably in step (e) the predetermined time period is up to 4 hours.

Preferably step (d) comprises heating the titanium aluminide alloy to a temperature about 30°C to 60°C below the alpha transus temperature.

Preferably step (a) comprises heating the titanium aluminide alloy to a temperature of about 20°C to 30°C above the alpha transus temperature.

Preferably step (f) comprises air-cooling or furnace cooling.

Preferably step (c) comprises air-cooling or oil cooling.

Preferably the titanium aluminide alloy consists of at least 46at% aluminium. The titanium aluminide alloy may comprise 48at% aluminium, 2at% chromium, 2at% niobium and the balance titanium and incidental impurities.

The alpha transus temperature is about 1360°C, step (a) comprises heating to a temperature of 1380°C, step (b) comprises maintaining the titanium aluminide alloy at a temperature of about 1380°C for about 1 hour, step (c) comprises oil cooling the titanium aluminide alloy from a temperature of 1380°C to produce a massively transformed gamma microstructure, steps (d) and (e) comprise heating the titanium aluminide alloy to a temperature of about 1320°C for about 2 hours to precipitate alpha plates in the massively transformed gamma microstructure such that a refined microstructure is produced in the titanium aluminide alloy, and step (f) comprises air cooling the titanium aluminide alloy to ambient temperature.

The titanium aluminide alloy may comprise 46at% aluminium, 8at% niobium, up to 0.07at% carbon and the balance titanium and incidental impurities.

The alpha transus temperature is about 1335°C, step (a) comprises heating to a temperature of 1360°C, step (b) comprises maintaining the titanium aluminide alloy at a temperature of about 1360°C for about 1 hour, step (c) comprises oil cooling, or air cooling, the titanium aluminide alloy from a temperature of 1360°C to produce a massively transformed gamma microstructure, steps (d) and (e) comprise heating the titanium aluminide alloy to a temperature of about 1300°C for about 4 hours to precipitate alpha plates in the massively transformed gamma microstructure such that a refined microstructure is produced in the titanium aluminide alloy, and step (f) comprises air cooling the titanium aluminide alloy to ambient temperature.

The present invention is applicable to a gamma titanium aluminide alloy consisting of 45-46at% aluminium, 8at% niobium, up to 0.07at% carbon and the balance titanium and incidental impurities, for example 45.5at% aluminium, 8at% niobium and the balance titanium and incidental impurities. The present invention is also applicable to a gamma titanium aluminide alloy consisting of 45-46at% aluminium, 2-6at% niobium, 2-6at% hafnium and the balance titanium and incidental impurities, for example 46at% aluminium, 4at% niobium, 4at% hafnium and the balance titanium and incidental impurities.

The titanium aluminide alloy may be a cast titanium aluminide component.

The method may comprise hot isostatic pressing of the cast titanium aluminide alloy component.

Preferably the hot isostatic pressing of the cast titanium aluminide alloy component is concurrent with step (e) .

Preferably the hot isostatic pressing comprises applying a pressure of about 150Mpa for about 4 hours.

The titanium aluminide alloy may be a compressor blade or a compressor vane.

The present invention will be more fully described by way of example with reference to the accompanying drawings in which:-
Figure 1 is graph of temperature versus time illustrating the method of heat-treating a titanium aluminide alloy according to the present invention.
Figure 2 is a schematic view of the microstructure of a titanium aluminide alloy heat treated according to the present invention.
Figure 3 is a view of the microstructure of a titanium aluminide alloy heat treated according to the present invention.
Figure 4 is a schematic view of the microstructure of a titanium aluminide alloy heat treated according to the prior art.
Figure 5 is a gamma titanium aluminide alloy gas turbine engine compressor blade heat treated according to the present invention.

A method of heat-treating a titanium aluminide alloy according to the present invention is described with reference to figure 1. The present invention is concerned with heat-treating gamma titanium aluminide alloys with at least 46at% aluminium and a single alpha phase field.

The heat treatment process comprises heating the gamma titanium aluminide to a temperature T₁ above the alpha transus temperature T_{α}. The gamma titanium aluminide alloy is then maintained at a temperature T₁ above the alpha transus temperature T_{α} in the single alpha phase field for a predetermined time period t₁. The gamma titanium aluminide is quenched, for example air cooled, or oil cooled, from the single alpha phase field at temperature T₁ to produce a massively transformed gamma microstructure. The gamma titanium aluminide alloy is then heated to a temperature T₂ below the alpha transus temperature T_{α}. The gamma titanium aluminide alloy is maintained at the temperature T₂ in the alpha and gamma phase field for a predetermined time period t₂ to precipitate alpha plates in the massively transformed gamma microstructure such that a refined microstructure is produced in the titanium aluminide alloy. The gamma titanium aluminide is cooled, for example air cooled, or furnace cooled, to ambient temperature.

Figure 2 illustrates a very fine duplex microstructure of a gamma titanium aluminide alloy treated according to the present invention. In the present invention differently orientated alpha plates precipitated in a massive gamma phase matrix effectively reduce the grain size of the gamma titanium aluminide alloy and these are produced by the massive gamma to alpha + gamma phase transformation.

For comparison Figure 4 illustrates a coarse lamellar microstructure of a gamma titanium aluminide alloy treated according to a prior art method. In the prior art the coarse lamellar microstructure is produced by the alpha to alpha + gamma phase transformation.

In particular, the gamma titanium aluminide is heated to a temperature T₁ about 20°C to 30°C above the alpha transus temperature T_{α}. The gamma titanium aluminide alloy is maintained at the temperature T₁ for up to 2 hours. The gamma titanium aluminide alloy is then quenched, for example air cooled, or oil cooled, at a rate sufficient to induce a massively transformed gamma microstructure. The gamma titanium alloy is heated to a temperature T₂ about 30°C to 60°C below the alpha transus temperature T_{α}. The gamma titanium aluminide alloy is maintained at the temperature T₂ for up to 4 hours to precipitate fine alpha plates with different orientations in the massively transformed gamma microstructure due to the massive gamma to alpha + gamma phase transformation. This gives rise to a very fine duplex microstructure. The differently orientated alpha plates precipitated in the massive gamma phase matrix effectively reduce the grain size of the gamma titanium aluminide. The gamma titanium aluminide alloy is then cooled, for example air cooled, or furnace cooled, to ambient temperature.

The holding at temperature T₁ for a time period t₁ also acts a homogenisation process for cast titanium aluminide alloys.

### Example 1

A gamma titanium aluminide alloy consisting of 48at% aluminium, 2at% chromium, 2at% niobium and the balance titanium plus incidental impurities was heat treated according to the present invention. This gamma titanium aluminide alloy has an alpha transus temperature T_{α} = 1360°C. The gamma titanium aluminide alloy was heated to a temperature T₁ = 1380°C and was held at T₁ = 1380°C for 1 hour. The gamma titanium aluminide alloy was oil cool quenched. The gamma titanium aluminide alloy was heated to a temperature T₂ = 1320°C and was held at T₂ = 1320°C for 2 hours. The gamma titanium aluminide alloy was air cooled to ambient temperature. The microstructure of the gamma titanium aluminide alloy is shown in figure 3.

### Example 2

A gamma titanium aluminide alloy consisting of 46at% aluminium, 8at% niobium, up to 0.07at% carbon and the balance titanium plus incidental impurities was heat treated according to the present invention. This gamma titanium aluminide alloy has an alpha transus temperature T_{α} = 1335°C. The gamma titanium aluminide alloy was heated to a temperature T₁ = 1360°C and was held at T₁ = 1360°C for 1 hour. The gamma titanium aluminide alloy was oil quenched. The gamma titanium aluminide alloy was heated to a temperature T₂ = 1300°C and was held at T₂ = 1300°C for 4 hours. The gamma titanium aluminide alloy was air cooled to ambient temperature.

The present invention is applicable to a gamma titanium aluminide alloy consisting of 46at% aluminium, 5at% niobium, 0.3at% boron, 0.2at% carbon and the balance titanium plus incidental impurities. The present invention is applicable to a gamma titanium aluminide alloy consisting of 47at% aluminium, 2at% niobium, 1at% tungsten, 1at% chromium, 1at% boron, 0.2at% silicon and the balance titanium plus incidental impurities. The present invention is applicable to gamma titanium aluminide alloy consisting of 47at% aluminium, 2at% tantalum, 1at% chromium, 1at% manganese, 1at% boron, 0.2at% silicon and the balance titanium plus incidental impurities. The present invention is also applicable to gamma titanium aluminide alloy consisting of 46at% aluminium, 5at% niobium, 1at% tungsten and the balance titanium plus incidental impurities.

The present invention is applicable to a gamma titanium aluminide alloy consisting of 45-46at% aluminium, 8at% niobium, up to 0.07at% carbon and the balance titanium and incidental impurities, for example 45.5at% aluminium, 8at% niobium and the balance titanium and incidental impurities. The present invention is also applicable to a gamma titanium aluminide alloy consisting of 45-46at% aluminium, 2-6at% niobium, 2-6at% hafnium and the balance titanium and incidental impurities, for example 46at% aluminium, 4at% niobium, 4at% hafnium and the balance titanium and incidental impurities.

The present invention may be used to refine the microstructure of titanium aluminide alloys without the need for hot working. The present invention has the advantage of simplicity and practicality over the prior art previously discussed. The heat treatment at temperature T₁ for time t₁ in the single alpha phase field and does not have a rigid holding time and this allows the process to be carried out in conventional heat treatment facilities. The gamma titanium aluminide alloys must be capable of producing massively transformed gamma microstructures. The cooling rate during the quenching is not excessive and most gamma titanium aluminide alloys with at least 46at% aluminium and with at least 4at% refractory alloying elements may be quenched in air or oil depending on the size of the gamma titanium aluminide alloy component. This significantly reduces the possibility of cracking of the gamma titanium aluminide alloy component during quenching. The temperature range for heat treatment at temperature T₂ for time t₂ is relatively wide and is not close to the alpha transus temperature T_{α}, which reduces the technical requirement of the heat treatment facilities and makes the heat treatment process easier. The present invention is particularly useful for gamma titanium aluminide alloy castings in which hot working is not possible. The present invention refines the microstructure of gamma titanium aluminide alloy castings and reduces the scatter in mechanical properties and improves the room temperature ductility.

In the case of cast gamma titanium aluminide alloy components it may be necessary to remove porosity from the cast gamma titanium aluminide alloy component. In this case the cast gamma titanium aluminide alloy component may be hot isostatically pressed (HIP) to remove the porosity. The hot isostatic pressing preferably occurs at the same time as the heat treatment temperature T₂ and for the time period of about 4 hours at a pressure of about 150Mpa and this is beneficial because this dispenses with the requirement for a separate hot isostatic pressing step.

The present invention is particularly suitable for gamma titanium aluminide gas turbine engine compressor blades as illustrated in figure 5. The compressor blade 10 comprises a root 12, a shank 14, a platform 16 and an aerofoil 18. The present invention is also suitable for gamma titanium aluminide gas turbine engine compressor vanes or other gamma titanium aluminide gas turbine engine components. The present invention may also be suitable for gamma titanium aluminide components for other engine, machines or applications.

## Claims

1. A method of heat-treating a titanium aluminide alloy, the titanium aluminide alloy having a single alpha phase field and being capable of producing a massively transformed gamma microstructure the method comprising the steps of
(a) heating a titanium aluminide alloy to a temperature above the alpha transus temperature,
(b) maintaining the titanium aluminide alloy at the temperature above the alpha transus temperature in the single alpha phase field for a predetermined time period,
(c) cooling the titanium aluminide alloy from the single alpha phase field to produce a massively transformed gamma microstructure,
(d) heating the titanium aluminide alloy to a temperature below the alpha transus temperature in the alpha and gamma phase field,
(e) maintaining the titanium aluminide alloy at the temperature below the alpha transus temperature for a predetermined time period to precipitate alpha plates in the massively transformed gamma microstructure such that a refined microstructure is produced in the titanium aluminide alloy,
(f) cooling the titanium aluminide alloy to ambient temperature.

2. A method as claimed in claim 1 wherein in step (b) the predetermined time period is up to 2 hours.

3. A method as claimed in claim 1 or claim 2 wherein in step (e) the predetermined time period is up to 4 hours.

4. A method as claimed in claim 1, claim 2 or claim 3 wherein step (d) comprises heating the titanium aluminide alloy to a temperature about 30°C to 60°C below the alpha transus temperature.

5. A method as claimed in any of claims 1 to 4 wherein step (a) comprises heating the titanium aluminide alloy to a temperature of about 20°C to 30°C above the alpha transus temperature.

6. A method as claimed in any of claims 1 to 5 wherein step (f) comprises air-cooling or furnace cooling.

7. A method as claimed in any of claims 1 to 6 wherein step (c) comprises air-cooling or oil cooling.

8. A method as claimed in any of claims 1 to 7 wherein the titanium aluminide alloy consists of at least 46at% aluminium.

9. A method as claimed in any of claims 1 to 8 wherein the titanium aluminide alloy comprises 48at% aluminium, 2at% chromium, 2at% niobium and the balance titanium and incidental impurities.

10. A method as claimed in claim 9 wherein the alpha transus temperature is about 1360°C, step (a) comprises heating to a temperature of 1380°C, step (b) comprises maintaining the titanium aluminide alloy at a temperature of about 1380°C for about 1 hour, step (c) comprises oil cooling the titanium aluminide alloy from a temperature of 1380°C to produce a massively transformed gamma microstructure, steps (d) and (e) comprise heating the titanium aluminide alloy to a temperature of about 1320°C for about 2 hours to precipitate alpha plates in the massively transformed gamma microstructure such that a refined microstructure is produced in the titanium aluminide alloy, and step (f) comprises air cooling the titanium aluminide alloy to ambient temperature.

11. A method as claimed in any of claims 1 to 8 wherein the titanium aluminide alloy comprises 46at% aluminium, 8at% niobium, up to 0.07at% carbon and the balance titanium and incidental impurities.

12. A method as claimed in claim 11 wherein the alpha transus temperature is about 1335°C, step (a) comprises heating to a temperature of 1360°C, step (b) comprises maintaining the titanium aluminide alloy at a temperature of about 1360°C for about 1 hour, step (c) comprises oil cooling, or air cooling, the titanium aluminide alloy from a temperature of 1360°C to produce a massively transformed gamma microstructure, steps (d) and (e) comprise heating the titanium aluminide alloy to a temperature of about 1300°C for about 4 hours to precipitate alpha plates in the massively transformed gamma microstructure such that a refined microstructure is produced in the titanium aluminide alloy, and step (f) comprises air cooling the titanium aluminide alloy to ambient temperature.

13. A method as claimed in any of claims 1 to 7 wherein the titanium aluminide alloy consists of 45-46at% aluminium, 8at% niobium, up to 0.07at% carbon and the balance titanium and incidental impurities.

14. A method as claimed in any of claims 1 to 7 wherein the titanium aluminide alloy consists of 45-46at% aluminium, 2-6at% niobium, 2-6at% hafnium and the balance titanium and incidental impurities.

15. A method as claimed in claim 14 wherein the titanium aluminide alloy consists of 46at% aluminium, 4at% niobium, 4at% hafnium and the balance titanium and incidental impurities.

16. A method as claimed in any of claims 1 to 15 wherein the titanium aluminide alloy is a cast titanium aluminide alloy component.

17. A method as claimed in claim 16 comprising hot isostatic pressing of the cast titanium aluminide alloy component.

18. A method as claimed in claim 17 wherein the hot isostatic pressing of the cast titanium aluminide alloy component is concurrent with step (e).

19. A method as claimed in claim 17 or claim 18 wherein the hot isostatic pressing comprises applying a pressure of about 150MPa for about 4 hours.

20. A method as claimed in any of claims 1 to 19 wherein the titanium aluminide alloy is a compressor blade or a compressor vane.

## Patentansprüche

1. Verfahren zur Wärmebehandlung einer Titanaluminid-Legierung, wobei die Titanaluminid-Legierung ein Alpha-Einphasenfeld aufweist und in der Lage ist, eine massiv transformierte Gamma-Mikrostruktur zu erzeugen, wobei das Verfahren die folgenden Schritte aufweist:
(a) es wird die Titanaluminid-Legierung auf eine Temperatur über der Alpha-Übergangstemperatur erhitzt;
(b) es wird die Titanaluminid-Legierung auf einer Temperatur über der Alpha-Übergangstemperatur im Alpha-Einphasenfeld eine vorbestimmte Zeitdauer lang gehalten;
(c) es wird die Titanaluminid-Legierung aus dem Alpha-Einphasenfeld abgekühlt, um eine massiv transformierte Gamma-Mikrostruktur zu erzeugen;
(d) es wird die Titanaluminid-Legierung auf eine Temperatur unter der Alpha-Übergangstemperatur im Alpha-Phasenfeld und im Gamma-Phasenfeld erhitzt;
(e) es wird die Titanaluminid-Legierung auf der Temperatur unter der Alpha-Übergangstemperatur eine vorbestimmte Zeitdauer lang gehalten, um Alpha-Plättchen in der massiv transformierten Gamma-Mikrostruktur auszufällen, so dass eine verfeinerte Mikrostruktur in der Titanaluminid-Legierung erhalten wird;
(f) es wird die Titanaluminid-Legierung auf Umgebungstemperatur abgekühlt.

2. Verfahren nach Anspruch 1, bei welchem im Schritt (b) die vorbestimmte Zeitdauer bis zu 2 Stunden beträgt.

3. Verfahren nach Anspruch 1 oder Anspruch 2, bei welchem im Schritt (e) die vorbestimmte Zeitdauer bis zu 4 Stunden beträgt.

4. Verfahren nach Anspruch 1, Anspruch 2 oder Anspruch 3, bei welchem der Schritt (d) die Erwärmung der Titanaluminid-Legierung auf eine Temperatur von etwa 30°C bis 60°C unter der Alpha-Übergangstemperatur umfasst.

5. Verfahren nach einem der Ansprüche 1 bis 4, bei welchem der Schritt (a) die Erwärmung der Titanaluminid-Legierung auf eine Temperatur von etwa 20°C bis 30°C über der Alpha-Übergangstemperatur umfasst.

6. Verfahren nach einem der Ansprüche 1 bis 5, bei welchem der Schritt (f) eine Luftabkühlung oder eine Ofenabkühlung umfasst.

7. Verfahren nach einem der Ansprüche 1 bis 6, bei welchem der Schritt (c) eine Luftabkühlung oder eine Ölabkühlung umfasst.

8. Verfahren nach einem der Ansprüche 1 bis 7, bei welchem die Titanaluminid-Legierung wenigstens 46at% Aluminium enthält.

9. Verfahren nach einem der Ansprüche 1 bis 8, bei welchem die Titanaluminid-Legierung 48at% Aluminium, 2at% Chrom, 2at% Niob und als Rest Titan und zufällige Verunreinigungen enthält.

10. Verfahren nach Anspruch 9, bei welchem die Alpha-Übergangstemperatur etwa 1360°C aufweist, bei welchem der Schritt (a) eine Erwärmung auf eine Temperatur von 1380°C aufweist, bei welchem der Schritt (b) eine Aufrechterhaltung der Titanaluminid-Legierung auf einer Temperatur von 1380°C für eine Zeitdauer von etwa 1 Stunde umfasst, bei welchem der Schritt (c) eine Ölabkühlung der Titanaluminid-Legierung von einer Temperatur von 1380°C umfasst, um eine massiv transformierte Gamma-Mikrostruktur zu erhalten, bei welchem die Schritte (d) und (e) eine Erwärmung der Titanaluminid-Legierung auf eine Temperatur von etwa 1320°C während etwa 2 Stunden umfassen, um Alpha-Plättchen in der massiv transformierten Gamma-Mikrostruktur auszufällen, so dass eine verfeinerte Mikrostruktur in der Titanaluminid-Legierung erzeugt wird und bei welchem der Schritt (f) eine Luftabkühlung der Titanaluminid-Legierung auf Umgebungstemperatur umfasst.

11. Verfahren nach einem der Ansprüche 1 bis 8, bei welchem die Titanaluminid-Legierung 46at% Aluminium, 8at% Niob, bis zu 0,07at% Kohlenstoff und als Rest Titan und zufällige Verunreinigungen enthält.

12. Verfahren nach Anspruch 11, bei welchem die Alpha-Übergangstemperatur bei etwa 1335°C liegt, bei welchem der Schritt (a) eine Erwärmung auf eine Temperatur von 1360°C umfasst, bei welchem der Schritt (b) eine Aufrechterhaltung der Titanaluminid-Legierung auf einer Temperatur von etwa 1360°C während etwa 1 Stunde umfasst, bei welchem der Schritt (c) eine Ölabkühlung oder eine Luftabkühlung der Titanaluminid-Legierung auf einer Temperatur von 1360°C umfasst, um eine massiv transformierte Gamma-Mikrostruktur zu erhalten, bei welchem die Schritte (d) und (e) eine Erwärmung der Titanaluminid-Legierung auf eine Temperatur von etwa 1300°C während etwa 4 Stunden umfassen, um die Alpha-Plättchen in der massiv transformierten Gamma-Mikrostruktur auszufällen, so dass eine verfeinerte Mikrostruktur in der Titanaluminid-Legierung erzeugt wird, und bei welchem der Schritt (f) eine Luftabkühlung der Titanaluminid-Legierung auf Umgebungstemperatur umfasst.

13. Verfahren nach einem der Ansprüche 1 bis 7, bei welchem die Titanaluminid-Legierung aus 45-46at% Aluminium, 8at% Niob, bis zu 0,07at% Kohlenstoff und als Rest aus Titan und zufälligen Verunreinigungen besteht.

14. Verfahren nach einem der Ansprüche 1 bis 7, bei welchem die Titanaluminid-Legierung aus 45-46at% Aluminium, 2-6at% Niob, 2-6at% Hafnium und als Rest aus Titan und zufälligen Verunreinigungen besteht.

15. Verfahren nach Anspruch 14, bei welchem die Titanaluminid-Legierung aus 46at% Aluminium, 4at% Niob, 4at% Hafnium und als Rest aus Titan und zufälligen Verunreinigungen besteht.

16. Verfahren nach einem der Ansprüche 1 bis 15, bei welchem die Titanaluminid-Legierung ein gegossenes Titanaluminid-Legierungs-Werkstück ist.

17. Verfahren nach Anspruch 16, bei welchem das gegossene Titanaluminid-Legierungs-Werkstück isostatisch heiß verpresst wird.

18. Verfahren nach Anspruch 17, bei welchem das heiße isostatische Verpressen des gegossenen Titanaluminid-Legierungs-Werkstücks gleichzeitig mit dem Schritt (e) geschieht.

19. Verfahren nach den Ansprüchen 17 oder 18, bei welchem das heiße isostatische Verpressen die Anwendung eines Druckes von etwa 150 Mpa während etwa 4 Stunden umfasst.

20. Verfahren nach einem der Ansprüche 1 bis 19, bei welchem die Titanaluminid-Legierung eine Kompressor-Laufschaufel oder eine Kompressor-Leitschaufel ist.

## Revendications

1. Procédé pour traiter thermiquement un alliage d'aluminure de titane, l'alliage d'aluminure de titane ayant un domaine de phase alpha unique et étant capable de produire une microstructure gamma massivement transformée, le procédé comprenant les étapes de :
(a) chauffer un alliage d'aluminure de titane à une température au-delà de la température de transus alpha,
(b) maintenir l'alliage d'aluminure de titane à la température au-delà de la température de transus alpha dans le domaine de phase alpha unique pour une période de temps prédéterminée,
(c) refroidir l'alliage d'aluminure de titane à partir du domaine de phase alpha unique pour produire une microstructure gamma massivement transformée,
(d) chauffer l'alliage d'aluminure de titane à une température inférieure à la température de transus alpha dans le domaine de phase alpha et gamma,
(e) maintenir l'alliage d'aluminure de titane à la température inférieure à la température de transus alpha pendant une période de temps prédéterminée pour précipiter des plaques alpha dans la microstructure gamma massivement transformée de telle sorte qu'une microstructure raffinée est produite dans l'alliage d'aluminure de titane,
(f) refroidir l'alliage d'aluminure de titane à la température ambiante.

2. Procédé selon la revendication 1, dans lequel dans l'étape (b) la période de temps prédéterminée va jusqu'à 2 heures.

3. Procédé selon la revendication 1 ou la revendication 2, dans lequel dans l'étape (e) la période de temps prédéterminée va jusqu'à 4 heures.

4. Procédé selon la revendication 1, la revendication 2 ou la revendication 3, dans lequel l'étape (d) comprend de chauffer l'alliage d'aluminure de titane à une température située d'environ 30°C à 60°C en dessous de la température de transus alpha.

5. Procédé selon l'une quelconque des revendications 1 à 4, dans lequel l'étape (a) comprend de chauffer l'alliage d'aluminure de titane à une température d'environ 20°C à 30°C au-dessus de la température de transus alpha.

6. Procédé selon l'une quelconque des revendications 1 à 5, dans lequel l'étape (f) comprend un refroidissement à air ou un refroidissement à four.

7. Procédé selon l'une quelconque des revendications 1 à 6, dans lequel l'étape (c) comprend un refroidissement à air ou un refroidissement à huile.

8. Procédé selon l'une quelconque des revendications 1 à 7, dans lequel l'alliage d'aluminure de titane comprend au moins 46% atomique d'aluminium.

9. Procédé selon l'une quelconque des revendications 1 à 8, dans lequel l'alliage d'aluminure de titane comprend 48% atomique d'aluminium, 2% atomique de chrome, 2% atomique de niobium et le reste de titane et d'impuretés incidentes.

10. Procédé selon la revendication 9, dans lequel la température de transus alpha est d'environ 1360°C, l'étape (a) comprend de chauffer à une température de 1380°C, l'étape (b) comprend de maintenir l'alliage d'aluminure de titane à une température d'environ 1 380°C pendant environ 1 heure, l'étape (c) comprend un refroidissement à huile de l'alliage d'aluminure de titane à partir d'une température de 1380°C pour produire une microstructure gamma massivement transformée, les étapes (d) et (e) comprennent de chauffer l'alliage d'aluminure de titane à une température d'environ 1 320°C pendant environ 2 heures pour précipiter des plaques alpha dans la microstructure gamma massivement transformée de telle sorte qu'une microstructure raffinée est produite dans l'alliage d'aluminure de titane, et l'étape (f) comprend de refroidir par air l'alliage d'aluminure de titane à la température ambiante.

11. Procédé selon l'une quelconque des revendications 1 à 8, dans lequel l'alliage d'aluminure de titane comprend 46% atomique d'aluminium, 8% atomique de niobium, jusqu'à 0,07% atomique de carbone et le reste de titane et d'impuretés incidentes.

12. Procédé selon la revendication 11, dans lequel la température de transus alpha est d'environ 1335°C, l'étape (a) comprend de chauffer à une température de 1360°C, l'étape (b) comprend de maintenir l'alliage d'aluminure de titane à une température d'environ 1 360°C pendant environ 1 heure, l'étape (c) comprend de refroidir par huile ou de refroidir par air, l'alliage d'aluminure de titane à partir d'une température de 1360°C pour produire une microstructure gamma massivement transformée, les étapes (d) et (e) comprennent de chauffer l'alliage d'aluminure de titane à une température d'environ 1 300°C pendant environ 4 heures pour précipiter des plaques alpha dans la microstructure gamma massivement transformée de telle sorte qu'une microstructure raffinée est produite dans l'alliage d'aluminure de titane, et l'étape (f) comprend de refroidir par air l'alliage d'aluminure de titane à la température ambiante.

13. Procédé selon l'une quelconque des revendications 1 à 7, dans lequel l'alliage d'aluminure de titane comprend 45-46% atomique d'aluminium, 8% atomique de niobium, jusqu'à 0,07% atomique de carbone et le reste de titane et d'impuretés incidentes.

14. Procédé selon l'une quelconque des revendications 1 à 7, dans lequel l'alliage d'aluminure de titane comprend 45-46% atomique d'aluminium, 2-6% atomique de niobium, 2-6% atomique d'hafnium et le reste de titane et d'impuretés incidentes.

15. Procédé selon la revendication 14, dans lequel l'alliage d'aluminure de titane comprend 46% atomique d'aluminium, 4% atomique de niobium, 4% atomique d'hafnium et le reste de titane et d'impuretés incidentes.

16. Procédé selon l'une quelconque des revendications 1 à 15, dans lequel l'alliage d'aluminure de titane est un composant d'alliage d'aluminure de titane de fonte.

17. Procédé selon la revendication 16, comprenant de comprimer de manière isostatique à chaud le composant d'alliage d'aluminure de titane de fonte.

18. Procédé selon la revendication 17, dans lequel la compression isostatique à chaud du composant d'alliage d'aluminure de titane de fonte est concomitante à l'étape (e).

19. Procédé selon la revendication 17 ou la revendication 18, dans lequel la compression isostatique à chaud comprend d'appliquer une pression d'environ 150MPa pendant environ 4 heures.

20. Procédé selon l'une quelconque des revendications 1 à 19, dans lequel l'alliage d'aluminure de titane est une pale de compresseur ou une aube de compresseur.
